

Patented Feb. 17, 1925.

1,526,620

## UNITED STATES PATENT OFFICE.

VICTOR YNGVE, OF SOUTH ORANGE, NEW JERSEY, AND CHARLES G. BIRDSALL, OF ELMHURST, NEW YORK, ASSIGNEES TO MANHATTAN ELECTRICAL SUPPLY COMPANY, INCORPORATED, OF NEW YORK, N. Y., A CORPORATION OF MASSACHUSETTS.

### METHOD OF MANUFACTURING DRY CELLS.

No Drawing.

Application filed March 28, 1924. Serial No. 702,583.

*To all whom it may concern:*

Be it known that we, VICTOR YNGVE and CHARLES G. BIRDSALL, citizens of the United States, residing at South Orange, in the county of Essex and State of New Jersey, and at Elmhurst, in the county of Queens and State of New York, respectively, have invented certain new and useful Improvements in Methods of Manufacturing Dry Cells, of which the following is a specification.

This invention relates to an improved method of manufacturing dry cells and more particularly to the manufacture of dry cells in which the depolarizing mixture is in the form of compacted tablets.

We have found that ageing the tablets will increase their structural strength, whereby the breakage incident to handling by means of automatic machinery may be materially reduced. The length of time during which the tablets are aged depends on the composition of the tablets, and upon atmospheric and temperature conditions. We have found that under normal conditions two to four hours' ageing will appreciably increase the strength of the tablets and that they will continue thus to improve over a relatively long period that may amount to several weeks. We have found also that the ageing process can be accelerated by subjecting the tablets to higher than room temperatures. Any increase in the temperature speeds up the hardening process, but temperatures of 75 to 140° F. were found best.

In order to speed up the manufacturing process, the tablets as they come from the press are passed by any suitable means, such as an endless belt, through an oven heated to the desired degree and are then transferred to the assembling machine. Instead of this method the tablets may be placed in the open in suitable containers and left there for the desired length of time. This time depends upon the composition of the tablets and the temperature, and in order to increase the speed of manufacture, the tablets are subjected to heat for about half an hour.

What we claim is:

1. The process of increasing the mechanical strength of depolarizing mixture for use in dry cells which consists in ageing the mixture.

2. The process of increasing the mechanical strength of tablets compacted of depolarizing mixture which consists in ageing such tablets for from ten hours to one week.

3. The process of increasing the mechanical strength of tablets compacted of depolarizing mixture, which consists in subjecting the tablets to higher than room temperatures for a certain period of time and then assembling a dry cell out of such tablets.

In testimony whereof, we have signed our names to this specification, this 27th day of March, 1924.

VICTOR YNGVE.  
CHARLES G. BIRDSALL.